

Aug. 17, 1943.

J. W. PROCTOR ET AL

2,327,332

TANK CONSTRUCTION

Filed Sept. 3, 1941

2 Sheets-Sheet 1



INVENTORS  
James W. Proctor  
Walter S. Allen  
BY  
Joseph C. Ryan  
ATTORNEY

Aug. 17, 1943.

J. W. PROCTOR ET AL

2,327,332

TANK CONSTRUCTION

Filed Sept. 3, 1941

2 Sheets-Sheet 2

Fig. 4



Fig. 6,



Fig. 5.



INVENTORS  
James W. Proctor  
Walter S. Allen  
BY  
Joseph C. Ryan  
ATTORNEY

## UNITED STATES PATENT OFFICE

2,327,332

## TANK CONSTRUCTION

James W. Proctor, Summit, N. J., and Walter S. Allen, Flushing, N. Y., assignors to General Chemical Company, New York, N. Y., a corporation of New York

Application September 3, 1941, Serial No. 409,334

3 Claims. (Cl. 220—1)

This invention relates to improvements in construction of metallic tanks employed for example for transportation or storage of corrosive liquids such as sulfuric acid.

Steel tanks used for shipment or storage of strong sulfuric acid are subjected to heavy corrosive action which causes contamination of the acid with dissolved iron and, more importantly, final deterioration of the tank. In the course of investigations leading to development of the present invention, we found that the major cause of high corrosion is the heating effect of sunlight on the film of acid which remains on the inside wall of a tank when the acid level is lowered or when the tank is emptied entirely. The absorption of heat from sunlight in such instances is sufficient to raise the temperature of the steel tank sides and top many degrees in excess of the outside atmospheric temperature. Our tests show that rate of steel corrosion is greatly accelerated as the temperature of the acid constituting the acid film is increased. For example, we have found that steel is corroded by 66° Bé. (93.19%) sulfuric acid (a usual strength at which sulfuric acid is stored or shipped) about twice as fast at temperature of about 150° F. as compared with say 100° F. These temperatures are representative of those existing on a summer day when a body of acid is being unloaded from a tank car. Often the temperature of the acid being unloaded is about 100° F., and we have observed that the temperature of the film of acid on the walls of the tank for some time after unloading may be as high as 150° F. The same temperature differentials are found also in a storage tank on a hot summer day after acid withdrawal. Another factor is the contact of moist air, from any source, with the acid film. This moisture dilutes the acid and liberates heat locally. Further, heating and dilution of the sulfuric acid film decreases viscosity, permitting the residual film to run down the sides of the tank around the rivet heads with increasing corrosion and formation of deep grooves. Tests show that at all temperatures the corrosion rate increases rapidly as 66° Bé. acid is diluted to about 63° Bé. (83.34%), the latter strength being taken as an example of the H<sub>2</sub>SO<sub>4</sub> strength resulting when a film of acid adhering to the inner wall of the tank becomes diluted by moisture in the air entering thru the tank dome during unloading. Taking 1 as a corrosion rate of 66° Bé. sulfuric acid at 100° F., at weaker concentration and varying temperatures, tests show the following:

| Bé. | Temperature | Corrosion rate | Temperature | Corrosion rate |
|-----|-------------|----------------|-------------|----------------|
|     |             |                |             |                |
| 5   | 66°         | 100            | 150         | 2              |
|     | 65°         | 100            | 150         | 3              |
|     | 64°         | 100            | 150         | 5.5            |
|     | 63°         | 100            | 150         | 7              |

Thus at temperature of about 150° F., corrosion rate of 63° Bé. acid is about seven times greater than 66° Bé. acid at 100° F.

The principal object of this invention is provision of tank construction which will reduce and minimize corrosion, lower replacement and maintenance costs, and make possible delivery of acid less contaminated with iron. More particularly, the invention aims to accomplish these ends by provision of tank construction which functions to keep the temperature of acid body in the tank as close to atmospheric temperature as feasible, to minimize the thickness of the acid film forming on the tank walls as the acid level is lowered, and to materially reduce the temperature of the acid constituting such film as compared with film temperatures arising in standard constructions. The objects and advantages of the invention will appear from consideration of the following description taken in connection with the accompanying drawings, in which

Fig. 1 is a vertical, longitudinal section of a tank car;

Fig. 2 is a horizontal section taken on line 2—2 of Fig. 1;

Fig. 3 is a vertical section taken on line 3—3 of Fig. 1;

Fig. 4 is a vertical section of a cylindrical storage tank taken on the line 4—4 of Fig. 5;

Fig. 5 is a horizontal section taken on line 5—5 of Fig. 4, and

Fig. 6 is a vertical section taken on the line 6—6 of Fig. 5.

Fig. 1 illustrates a tank car comprising a horizontal cylindrical steel shell 10, end heads 11, and dome 12, all of usual construction. Outside of shell 10, and suitably spaced from it for example by 3 or 4 inches, is a metallic hood-like shield 13 held in place, relative to the tank in approximately the relationship shown in Fig. 3, by brackets 16 spot-welded or riveted at one end to the outside of the tank and to the shield at the other. Preferably the shield extends the length of the tank as shown in Fig. 2, and the end edges of the shield are welded to the outer edges of semi-circular steel end plates 14; the

inner edges 26 of which are welded to the circumference of the tank heads 11. Thus the shield 14, the adjacent portion of the outside tank and end plates 13 form an air chamber 21 which, in the embodiment shown in Fig. 3, covers the upper half of the tank. The arrangement is such that the lower ends of chamber 21 are open to the atmosphere at 22. As shown in Figs. 1 and 3, there are provided at the top of chamber 21, slots 23 and 24 extending from the dome to the ends of the tank. The cut-out portions of the shield immediately adjacent the outer surface of the dome 12 are spot-welded thereto as at 25, so that any acid spilled during loading or unloading will run off the upper surface of the shield. Thus, air chamber 21 is open to the atmosphere at both lower edges and by way of longitudinal slots 23, 24 at the top.

As a general rule the lower half of car and truck tanks is cylindrical, and consequently the lower half of the outer tank surface is protected from the direct rays of the sun during the hotter part of the day. As a result, the lower half is appreciably cooler and our observations show that acid corrosion on the lower half of the tank is small. Hence, in the embodiment of Fig. 3 the shield 14 is brought down far enough on either side to cover only approximately the upper half of the tank. In some instances, however, it may be desirable to extend the lower horizontal edges of the shield below the position shown in Fig. 3 sufficient, for example, to envelop say the upper two-thirds area of the tank. If desired, the shield might also be made to cover the upper half or more of the tank end walls 11.

A further feature of the invention comprises provision on the inside wall of the tank of deflecting plates such as 28, 29 and 30. These plates (Figs. 1 and 3) extend horizontally the length of the side walls, the cross-sectional shape of the plates being such that the upper faces are inclined downwardly. Similar plates 31 extend across the tank heads 11. As shown particularly in Fig. 3, the arrangement is such that the drip-off edge 33 of a plate projects into the tank beyond the drip-off edge of the immediately subjacent plate. The purpose of the deflecting plates is to shunt away, from the inner side and end walls of the tank, the acid film flowing down the walls as the tank is emptied. Moisture drawn into the tank as it is being emptied results in a film of weaker acid which is more corrosive than the acid loaded into the tank. It is important to the service life of the tank that the quantity of this film in contact with the shell and rivet heads be kept at a minimum to prevent both corrosion and grooving. Shunting the descending film off the walls at suitable intervals, keeps the corrosive action at a minimum. Most of whatever corrosion does take place is thus transferred to the plates which may be readily replaced at small cost. In Fig. 3, reference numeral 35 indicates a double horizontal row of rivets, and in this instance deflecting plates 30 are located directly above the line of riveting to minimize grooving around the rivet heads.

Figs. 4, 5 and 6 illustrate application of the invention to stationary storage tanks. In this modification, a cylindrical shield 40 extends completely around the circumference of tank 41, the shield being held suitably spaced from the outer wall 43 of the tank by a series of brackets 44 preferably spot-welded to the tank and riveted to the shield at 45. The annular air chamber 46 formed by the outer wall of the tank and the inner wall

of the shield 40 is open to the atmosphere at the top as at 51, and at the bottom communicates with the atmosphere thru a series of ports 54.

In Fig. 4, 55 and 56 indicate horizontal and vertical series of rivets. To afford protection for the riveting from the corrosive action of the acid film left on the inner walls of the tank when the acid is withdrawn, a horizontal deflecting plate 60 is fixed to the inner tank wall just above the line of riveting 55. At suitably spaced vertical intervals, other deflecting plates 61 are attached to the tank wall in the line of vertical riveting 56, as indicated in Fig. 6 which also shows that the drip-off edge, e. g. 64, of a given plate overhangs the drip-off edge of the subjacent plate.

In the car construction of Figs. 1-3, shield 14 is extended all the way over the top of the tank because when loaded, such tanks are completely filled, the acid usually rising a few inches in the dome. In the storage tank of Figs. 4-6, no shield is placed over the top since in practice it is not customary to entirely fill the tank, and there is no acid in direct contact with the metallic upper end of the tank.

In both embodiments illustrated in the drawings, atmospheric air is drawn in at the bottom of the chamber, formed by the shield and the outside of the tank, circulates freely up thru the chamber, and is discharged at the top. The heat of the sun striking the shield is largely dissipated by the atmospheric air passed thru the chamber by the chimney effect, and when the tank is filled or partly so, the construction described effects maintenance of temperatures of the acid in the tank substantially the same as the average temperature of the surrounding atmosphere. Such temperature control results in marked lower corrosion. The following data show the difference in corrosion effected in shaded and non-shaded tanks. Four horizontal cylindrical steel tanks were filled with 68° Bé. sulfuric acid containing .0003% iron, temperature of the acid on filling being 30° F. During a period of four days two of the tanks were shaded and two were left in the open exposed to the rays of the sun. Once a day, when temperature was maximum temperatures (1) of the atmosphere immediately adjacent the tank surfaces, (2) of the acid directly in contact with the tank surfaces, and (3) of the acid in the center of the tanks were taken. After the third day the acid in each tank was blown with air to mix the acid well and representative samples tested for iron, results being as follows:

|                              | In sun  | In sun  | In shade | In shade |         |
|------------------------------|---------|---------|----------|----------|---------|
| Temp. outside metal.         | °F. 110 | °F. 109 | °F. 80   | °F. 80   |         |
| Temp. acid next metal.       | 84      | 84      | 73       | 71       | Noon    |
| Temp. acid at center.        | 77      | 77      | 70       | 70       |         |
| Temp. outside metal.         | 123     | 121     | 85       | 85       |         |
| Temp. acid next metal.       | 93      | 97      | 74       | 75       | 1 P. M. |
| Temp. acid at center.        | 84      | 84      | 72       | 72       |         |
| Temp. outside metal.         | 76      | 76      | 72       | 72       |         |
| Temp. acid next metal.       | 77      | 77      | 72       | 72       | Noon    |
| Temp. acid at center.        | 74      | 74      | 72       | 72       |         |
| Percent Feinacid after test. | .0094   | .0086   | .0044    | .0048    |         |

The above tests show twice as much iron is dissolved when the tank is left in the sunlight. In the case of the tanks exposed to the sun,

the amount of iron dissolved corresponds with a corrosion rate of about .018 inch penetration per year.

A second and more important advantage of the construction of the invention is the cooperative result afforded by the shield and the deflecting plates. Temperature differences in tanks which have been emptied of acid and are in transit or in dead storage in the sunlight are much more pronounced than in the case of tanks which are filled. In numerous instances temperatures as high as 130° F. have been observed in empty acid tanks in the sunlight. Corrosion rate at 130° F. is approximately four times as great with 66° Bé. acid, as at temperature of about 70° F. This much higher rate of corrosion is caused first, by the much higher temperatures prevalent in an emptied tank and, second, by the film of acid, usually diluted by atmospheric moisture, which adheres to the tank sides after emptying. In the construction illustrated, the deflecting plates keep the thickness of the residual acid film on the inner walls of the tank at a minimum, and this feature in combination with the low temperatures maintained by the chimney effect created by the shield hold corrosion at a low point.

The shielding afforded by the invention should be distinguished from ordinary insulation. The latter tends to keep the contents of a tank at uniform temperature which will be approximately the temperature of the acid at the time of loading. The shielding provided by the present invention affords a maximum cooling of the contents after the tank is loaded. Because of plant operating requirements, a car or storage tank is often loaded with warm acid, for example 66° Bé. sulfuric acid at temperature of about 120° F. Corrosion caused by acid of this strength and temperature is at a rate of about .026 inch per year. Insulation merely holds this temperature at about 120° F. and corrosion proceeds at the accelerated rate indicated. By means of the chimney effect produced by the shielding of this invention, air currents are continually drawn up from the cooler layers of air on the ground, and cool the acid in the tank with resulting corrosion decrease. The construction of the invention provides active cooling at all seasons of the year, a phenomenon not afforded by the usual type of dead insulation. Further, the vigorous air movement up under the shield is effective in preventing temperature rise.

We claim:

1. A tank car comprising a horizontally disposed tank adapted to receive a corrosive liquid and made of material corrodible by said liquid and provided on top with a centrally located dome, a hood-like shield extending the length of the tank and substantially covering the outer wall of at least the upper half of the tank, end plates connecting the end edges of said shield with the adjacent circumferences of the ends of the tank, said shield being spaced from such outer wall of said tank and forming, with said

end plates, an air chamber between such outer wall of said tank and the inner wall of said shield, contiguous portions of said shield and said dome being associated in liquid-tight relation, elongated openings at the bottom of said chamber on either side of the tank for ingress of atmospheric air, and slots extending from said dome to either end of the tank at the top of said chamber for egress of such air after upward passage through said chamber.

2. A tank car comprising a horizontally disposed tank adapted to receive a corrosive liquid and made of material corrodible by said liquid and provided on top with a centrally located dome, a hood-like shield extending the length of the tank and substantially covering the outer wall of at least the upper half of the tank, end plates connecting the end edges of said shield with the adjacent circumferences of the ends of the tank, said shield being spaced from such outer wall of said tank and forming, with said end plates, an air chamber between such outer wall of said tank and the inner wall of said shield, contiguous portions of said shield and said dome being associated in liquid-tight relation, elongated openings at the bottom of said chamber on either side of the tank for ingress of atmospheric air, slots extending from said dome to either end of the tank at the top of said chamber for egress of such air after upward passage through said chamber, a plurality of vertically spaced, horizontally disposed and downwardly inclined deflecting plates extending substantially the length of said tank, said plates being fixed to the inner wall of the upper half of said tank and arranged so that the drip-off edge of one plate projects into the tank beyond the drip-off edge of the immediately subjacent plates, said plates thereby effecting shunting from said inner wall surface of corrosive liquid flowing down said inner tank wall surface after the level of liquid in said tank has been lowered below a plate by withdrawal of liquid from said tank.

3. A tank car comprising a horizontally disposed tank adapted to receive a corrosive liquid and made of material corrodible by said liquid and provided on top with a centrally located dome, a hood-like shield extending the length of the tank and substantially covering the outer wall of at least the upper half of the tank, means connecting the end edges of said shield with the adjacent circumferences of the ends of the tank, said shield being spaced from such outer wall of said tank and forming an air chamber between such outer wall of said tank and the inner wall of said shield, elongated openings at the bottom of said chamber on either side of the tank for ingress of atmospheric air, and slots extending from said dome to either end of the tank at the top of said chamber for egress of such air after upward passage through said chamber.

JAMES W. PROCTOR.  
WALTER S. ALLEN.